

# United States Patent [19]

Dunbar et al.

[11] 3,926,572

[45] Dec. 16, 1975

[54] ALUMINIZED STEEL

3,058,206 10/1962 Mets ..... 29/196.2

[75] Inventors: **Frank C. Dunbar**, Monroe; **Kasimir Oganowski**, Middletown, both of Ohio

*Primary Examiner*—L. Dewayne Rutledge

*Assistant Examiner*—O. F. Crutchfield

[73] Assignee: **Armco Steel Corporation**, Middletown, Ohio

*Attorney, Agent, or Firm*—Melville, Strasser, Foster & Hoffman

[22] Filed: Aug. 29, 1974

[21] Appl. No.: 501,765

## [57] ABSTRACT

### Related U.S. Application Data

[63] Continuation of Ser. No. 320,523, Jan. 2, 1973, abandoned.

Steel base strip hot dip coated with substantially pure aluminum and adapted for porcelain enameling characterized by excellent reverse bend adherence. The interface iron-aluminum alloy must be less than about 0.45 ounces per square foot of sheet, and the free aluminum above the alloy layer must be in the range of 0.10 to 0.25 ounces per square foot of sheet.

### [56] References Cited

### UNITED STATES PATENTS

2,883,739 4/1959 Russell ..... 29/196.2

7 Claims, No Drawings

## ALUMINIZED STEEL

## Cross Reference To Related Application

This is a continuation of application Ser. No. 320,523 filed Jan. 2, 1973 and now abandoned.

## BACKGROUND OF THE INVENTION

This invention relates to a coated steel substrate particularly adapted for porcelain enameling. Porcelain enamel (sometimes called vitreous enamel) is a fired-on opaque glassy coating applied to steel for use in a variety of end products.

Most porcelain enameling to date has been carried out on plain steel or iron substrates. Since porcelain enameling is characterized by minute pinholes, the enameling is typically a multistage process, in that a plurality of layers of enamel will be fired on top of each other. Thus, the steel substrate is completely protected from corrosion.

It was later recognized that a steel substrate coated with a corrosion-resistant metal would be advantageous in porcelain enameling processes. Under these circumstances, the thickness of the porcelain enameling could be substantially reduced in that moisture or the like passing through pinholes in the porcelain coating would be stopped by the metallic coating. Similarly, the protective metallic coating makes it possible to porcelain enamel one side only for decorative purposes.

Further, the industry has recognized that aluminum is the preferred coating metal for subsequent porcelain enameling, because it offers excellent corrosion protection of the base steel and it is compatible with low temperature enameling processes resulting in a more ductile, adherent product.

Most commercially available aluminum coatings today are applied by a hot dip process wherein a strand is subjected to various pretreatments and then passed into a bath of molten aluminum. Typically, the molten aluminum will contain approximately ten percent silicon alloyed with the aluminum. In order to porcelain enamel such stock, it is necessary to first prefire the aluminum coated steel. The precise influence mechanism of this prefire is not fully known. It is, however, known that attempts to porcelain enamel directly over a silicon bearing aluminum coating usually results in a severe blistering. Prefiring at a temperature on the order of 1,000° F. is effective to eliminate the blistering problem.

It has also been known that blistering does not occur in the case of a pure aluminum coating; that is, an aluminum coating containing no silicon alloy. Therefore, a steel substrate coated with substantially pure aluminum does not require prefire in order to successfully receive a porcelain enamel coating.

However, the art has been unsuccessful in its attempts to produce a steel substrate having a pure aluminum coating which has good reverse bend adherence and which will not delaminate from the steel base during heating to a temperature of 1,000° F. In other words, the application of a porcelain enamel coating requires heating to temperatures on the order of 1,000° F. for 2-6 minutes. After this thermal cycling, the art has found that a steel substrate coated with substantially pure aluminum has a tendency for gross coating delamination.

Keeping the above comments in mind, it is a primary object of this invention to provide an aluminum coated steel substrate particularly suitable for porcelain enameling.

More specifically, it is an object of this invention to provide an aluminized steel for porcelain enameling which is characterized by excellent reverse bend adherence and eliminates the coating delamination hazard normally experienced during firing.

It is of course an object of this invention to provide an aluminized steel for porcelain enameling which does not require prefire to avoid enamel blistering.

## SUMMARY OF THE INVENTION

Broadly considered, this invention relates to a steel base strip coated with substantially pure aluminum and particularly adapted for porcelain enameling. The product is characterized by excellent reverse bend adherence and resistance to coating delamination during firing of the porcelain enamel.

As just indicated, the coating metal must be substantially pure aluminum, and preferably will be applied by a continuous hot dip coating process.

The process is controlled so that the weight of the interface iron aluminum alloy will be less than about 0.45 ounces per square foot of coated sheet. The layer of free aluminum above the alloy layer must be continuous without alloy "burn through," beyond this limit, the free aluminum layer should be as thin as possible.

Investigations have established that the free aluminum layer should be in the range of 0.10 to 0.25 ounces per square foot of coated sheet. In any event, total coating weight must be less than about 0.60 ounces per square foot of coated sheet.

## DESCRIPTION OF THE PREFERRED EMBODIMENT

As previously indicated, this invention relates to an aluminized steel; that is, a steel base strand coated with substantially pure aluminum. This aluminum coating may be applied by any of the many, well known continuous hot dip coating processes.

A typical hot dip coating process contemplates the rapid heating of a base steel strand in a non-oxidizing atmosphere so as to rapidly burn oil and the like from the surface of the strip. This is followed by continued heating in a reducing atmosphere, which is followed in turn by controlled cooling to bring the strip down to a temperature at or near the temperature of the molten aluminum. The strip is then passed into the molten aluminum bath and withdrawn therefrom in a generally vertical path of travel. The molten aluminum withdrawn from the bath by the moving strand will be finished with a jet air knife in accordance with the now well known techniques.

It is well known from prior experience that while the steel is in contact with molten aluminum, an interface iron aluminum alloy tends to form. On top of this interface alloy will be a layer of free or unalloyed aluminum.

The essence of this invention appears to lie in the thickness of these layers; that is, the thickness of the interface alloy layer and the thickness of the free aluminum layer above the alloy.

It is important to this invention that the interface iron aluminum alloy layer be less than about 0.45 ounces per square foot of coated sheet, and preferably should be less than about 0.35 ounces per square foot of coated sheet. (In accordance with industry convention,

the figures in terms of ounces per square foot relate to both sides of a coated strip.)

It is believed that the addition of silicon to the aluminum coating metal tends to retard the formation of this iron aluminum interface alloy. Thus, microscopic examination in cross section at 500X of a ferrous base strand coated with an aluminum silicon alloy will disclose a rather smooth boundary line between the iron and the alloy, and will further show a very thin interface alloy level.

By comparison, microscopic examination at the same magnification of a section of ferrous strand coated with substantially pure aluminum will usually show a "dog-tooth" or jagged, nonuniform boundary between the iron and the coating alloy layer. Similarly, the alloy layer is relatively much thicker.

It is very important to this invention that the free aluminum layer above the interface alloy be continuous. In other words, the free aluminum must be thick enough to prevent contact between the alloy layer and the applied porcelain enamel coating. With this limitation, the free aluminum layer should be as thin as possible.

Empirical investigations have disclosed that the free aluminum layer on top of the alloy layer should be on the order of 0.10 to 0.25 ounces per square foot of coated sheet.

It will be apparent from the foregoing that the total coating weight should be less than about 0.60 ounces per square foot.

A steel base strand with an aluminum coating having these characteristics has been commercially produced on a coating line conforming to that generally described earlier in this specification. The speed of the base strand through the coating metal bath varies between 120 and 450 feet per minute. This results in an immersion time in molten aluminum of from approximately 1.6 seconds to approximately 6 seconds.

The molten aluminum bath was maintained at a temperature of approximately 1,280° F., and the strip, after heating in the reducing atmosphere, was cooled to a temperature of approximately 1,200° F. to 1,250° F. prior to passage into the bath.

It is believed that the foregoing constitutes a full and complete disclosure of this invention, and no limitations are intended except insofar as specifically set forth in the claims which follow.

The embodiments of the invention in which an exclusive property of privilege is claimed are defined as follows:

5 1. A steel base sheet hot dip coated with a coating consisting essentially of substantially pure aluminum, said aluminum coated sheet having excellent reverse bend coating adherence and exhibiting no coating delamination during heating to a temperature on the order of 1,000° F., said coated sheet being characterized by an interface iron-aluminum alloy layer having a weight less than 0.45 ounces per square foot of coated sheet, and a continuous layer of unalloyed aluminum above said alloy layer, said unalloyed aluminum layer having a weight in the range of 0.10 to 0.25 ounces per 10 square foot of coated sheet, the total weight of said interface iron-aluminum alloy layer and said unalloyed aluminum layer being less than about 0.60 ounces per square foot of coated sheet, whereby to provide an aluminized steel base sheet particularly suitable for enamel coating.

15 2. The product claimed in claim 1 wherein the weight of said alloy layer is less than 0.35 ounces per square foot of coated sheet.

20 3. A steel base sheet hot dip coated with a coating consisting essentially of substantially pure aluminum, said aluminum coated sheet having excellent reverse bend coating adherence and exhibiting no coating delamination during heating to a temperature on the order of 1,000° F., said coated sheet being characterized by an interface iron-aluminum alloy layer on each side of said sheet, and a continuous layer of unalloyed aluminum above said alloy layer, the total weight of said alloy layer and said unalloyed aluminum layer being less than 0.60 ounces per square foot of coated sheet.

25 4. The product claimed in claim 3 wherein the weight of said unalloyed aluminum layer is less than 0.25 ounces per square foot of coated sheet.

30 5. The product claimed in claim 3 wherein the weight of said unalloyed aluminum layer is in the range of 0.10 to 0.25 ounces per square foot of coated sheet.

35 6. The product claimed in claim 3 wherein the weight of said alloy is less than 0.45 ounces per square foot of coated sheet.

40 7. The product claimed in claim 3 wherein the weight of said alloy layer is less than 0.35 ounces per square foot of coated sheet.

\* \* \* \* \*